

## UNITED STATES PATENT OFFICE

2,222,532

## SHEET MATERIAL

John Eggert, Leipzig-Gohlis, and Bruno Wendt,  
Dessau in Anhalt, Germany, assignors, by mesne  
assignments, to Walther H. Duisberg, New York,  
N. Y.

No Drawing. Application March 8, 1934, Serial  
No. 714,728. In Germany March 11, 1933

14 Claims.

(Cl. 91—68)

Our present invention relates to and one of its objects is an improved protective envelope for goods of any kind capable of being affected by light and air, such as victuals, books, textile fabrics or the like.

It has already been proposed to render impervious to ultra-violet rays envelopes consisting of sheets of paper, regenerated cellulose, superficially saponified cellulose acetate or the like by impregnating them with aesculin and

and 3,6-diaminocarbazole disulfonic acid, corresponding with the formula



(2) The sodium salt of 4,4'-tetramethyldiaminodibenzoyl-4,4'-diamino-diphenyl-2,2'-disulfonic acid corresponding with the formula

10



15

15

quinine sulfate. The protective envelopes prepared in this manner, however, have the drawback that the substances incorporated in them are eliminated by the action of moisture. Thus it happens, for instance, that by the moisture of victuals wrapped in envelopes of such kind, part of the incorporated substance is transferred to the victuals.

According to this invention the aforesaid drawback is avoided by incorporating in the envelopes a substance which has not only the required optical properties, but also has a substantive character and therefore has so strong an affinity to the sheet material from which the protective envelopes have been produced that it is no longer removed by moisture. The envelopes may be made from sheets of cellulose hydrate, paper, parchment, cellulose derivatives or the like. As compounds which have the required properties for instance, the following are suitable:

(1) The diaminodibenzoyl compounds of p-phenylenediamine disulfonic acid, corresponding with the formula



p-phenylenediamine sulfonic acid corresponding with the formula



or a substitution product thereof, for instance, the dianisidine disulfonic acid derivatives,

(3) The arylides of 2,3-hydroxynaphthoic acid corresponding with the formula

20



25

and derivatives, for instance



30



35

and the arylides of 2,3-hydroxynaphthoic-amino-sulfonic acid,

(4) Salicyl-p'-aminosalicyloyl-m''-aminophenol corresponding with the formula

40



45

(5) 3-hydroxydiphenylamine, corresponding with the formula

50



(6) The m-aminoanilide of 3-hydroxy-4-

55

chlorodiphenylamine carboxylic acid, corresponding with the formula



(7) (1,2,5-trichlorobenzene-4-sulfo)-(4',6'- dichloro-1'-phenol-2'-sulfo)-1''-3'' phenylenediamine corresponding with the formula



15 (8) 4-chloro-1-phenol-2,6-disulfo - bis -3'-ace-



25 tylamide-1'-anilide corresponding with the formula



35 All compounds enumerated are suitable for use with sheets made from cellulose for instance, paper or parchment or for use with sheets from cellulose hydrate or from gelatin. The 2,3-hydroxynaphthoic-amino sulfonic acid is also suitable for use with sheets from cellulose acetate.

If required, the sheets having incorporated in them colored or colorless substances absorbing 40 ultra-violet rays, may also receive an addition of a substance preventing oxidation of the first named substance, for instance, hydroquinone.

The following examples illustrate the invention:

45 Example 1.—A sheet of cellulose hydrate is soaked with an aqueous solution of 2 to 5 per cent strength of the sodium salt of the urea of p - aminobenzoyl-p-phenylenediaminosulfonic acid corresponding with the formula:



60 at a temperature of 50° C. If required the solution may contain an addition of 1 to 5 per cent. 60 of hydroquinone. If desired the sheet may be after-treated with glycerine for increasing flexibility.

Example 2.—A sheet of cellulose hydrate is soaked with an aqueous solution of the sodium 65 salt of di-m-aminobenzoyl-diaminostilbenedisulfonic acid, corresponding with the formula



washed with water and subsequently treated in a glycerin bath.

Example 3.—Pergamyne paper is treated with a 75 solution of the sodium salt of 4,4'-di-(p-amino-

benzoylamino) -diphenyl-2,2'-disulfonic acid corresponding with the formula



of 0.5 per cent strength for about 5 minutes at room temperature, and is then washed and dried. Instead of the 2,2'-disulfonic acid there may also 10 be used the 3,3'-disulfonic acid, the corresponding carboxyl acids and the compounds in which the hydrogen atoms of the amino groups are exchanged for alkyl.

Example 4.—To the paper pulp there is added 15 a solution of the sodium salt of the tetramethyl-diaminodibenzoyl compound of dianisidinedisulfonic acid corresponding with the formula



25 After the compound has been absorbed the mass is made into paper in the usual way.

Example 5.—A sheet of cellulose hydrate is treated with a solution of the sodium salt of 4,4'-tetramethyl-diaminodibenzoyl-4,4'-benzidine-2,2'-disulfonic acid of 0.5 per cent strength 30 for about 3 minutes at 80° C. The material is then washed and dried.

Example 6.—A solution of gelatin of 10 per cent strength is mixed with a solution of caustic alkali of 0.5 per cent strength containing 10 per 35 cent of the weight of the gelatin used of 2,3-hydroxynaphthoic-amino sulfonic acid- $\alpha$ -naphthalide corresponding with the formula



45 The solution is then caused to solidify and washed with water. The gelatin obtained is mixed with three times its weight of untreated gelatin and made into sheets.

What we claim is:

1. A process of producing a wrapping material which comprises incorporating in a sheet of cellulose hydrate the sodium salt of the urea of p-aminobenzoyl-p-phenylenediamine sulfonic acid corresponding with the formula



2. A process of producing a wrapping material which comprises incorporating in a sheet of gelatin 65 2,3-hydroxynaphthoic-amino sulfonic acid- $\alpha$ -naphthalide corresponding with the formula



3. A process of producing a wrapping material which comprises incorporating in a sheet of cellulose hydrate the tetramethyl-diaminodibenzoyl

compound of benzidine-2,2'-disulfonic acid corresponding with the formula



10 4. A sheet of cellulose hydrate containing the sodium salt of the urea of p-aminobenzoyl-p-phenylenediamine sulfonic acid corresponding with the formula



20 5. A sheet of gelatin containing 2,3-hydroxy-naphthoic-aminosulfonic acid- $\alpha$ -naphthalide corresponding with the formula



25 6. A sheet of cellulose hydrate containing the tetramethyldiaminodibenzoyl compound of benzidine-2,2'-disulfonic acid corresponding with the formula



35 7. A process of producing a wrapping material which comprises incorporating in a sheet material permeable to ultra violet rays a compound, substantive to said sheet material, selected from the class consisting of diaminodibenzoyl compounds of p-phenylenediamine disulfonic acid, p-phenylenediamine sulfonic acid and 3,6-diaminocarbazole disulfonic acid, the sodium salt of 4,4'-tetramethyldiamino-dibenzoyl-4,4'-diaminodiphenyl-2,2' disulfonic acid and substitution products thereof, the sodium salt of di-m-amino-benzoyl-diaminostilbene disulfonic acid, the arylides of 2,3-hydroxynaphthoic acid, the arylides of 2,3-hydroxynaphthoic-aminosulfonic acid, salicyl-p'-aminosalicyloyl-m''-aminophenol, 3-hydroxy-diphenylamine, m-aminoanilide of 3-hydroxy-4'-chlorodiphenylamine carboxylic acid, (1,2,5-trichlorobenzene-4-sulfo)-(4',6'-dichloro-1'-phenol-2'-sulfo)-1',3''-phenylenediamine, and 4-chloro-1-phenol-2,6-disulfo-bis-3'-acetylamide-1'-anilide in sufficient amount to effectively absorb ultra-violet rays.

8. A process of producing a wrapping material which comprises incorporating in a sheet material permeable to ultra violet rays a substance preventing oxidation and a compound, substantive to said sheet material, selected from the class consisting of diaminodibenzoyl compounds of p-phenylenediamine disulfonic acid, p-phenylenediamine sulfonic acid and 3,6-diaminocarbazole disulfonic acid, the sodium salt of 4,4'-tetramethyldiamino-dibenzoyl-4,4'-diamino-diphenyl-2,2' disulfonic acid and substitution products thereof, the sodium salt of di-m-amino-benzoyl-diaminostilbene disulfonic acid, the arylides of 2,3-hydroxynaphthoic acid, the arylides of 2,3-hydroxynaphthoic-aminosulfonic acid, salicyl-p'-aminosalicyloyl-m''-aminophenol, 3-

hydroxy-diphenylamine, m-aminoanilide of 3-hydroxy-4'-chlorodiphenylamine carboxylic acid, (1,2,5-trichlorobenzene-4-sulfo)-(4',6'-dichloro-1'-phenol-2'-sulfo)-1',3''-phenylenediamine, and 4-chloro-1-phenol-2,6-disulfo-bis-3'-acetylamide-1'-anilide in sufficient amount to effectively absorb ultra-violet rays.

10 9. A sheet material permeable to ultra violet rays containing a compound, substantive to said sheet material, selected from the class consisting of diaminodibenzoyl compounds of p-phenylenediamine disulfonic acid, p-phenylenediamine sulfonic acid and 3,6-diaminocarbazole disulfonic acid, the sodium salt of 4,4'-tetramethyldiamino-dibenzoyl-4,4'-diamino-diphenyl-2,2' disulfonic acid and substitution products thereof, the sodium salt of di-m-amino-benzoyl-diaminostilbene disulfonic acid, the arylides of 2,3-hydroxynaphthoic acid, the arylides of 2,3-hydroxynaphthoic-aminosulfonic acid, salicyl-p'-aminosalicyloyl-m''-aminophenol, 3-hydroxy-diphenylamine, m-aminoanilide of 3-hydroxy-4'-chlorodiphenylamine carboxylic acid, (1,2,5-trichlorobenzene-4-sulfo)-(4',6'-dichloro-1'-phenol-2'-sulfo)-1',3''-phenylenediamine, and 4-chloro-1-phenol-2,6-disulfo-bis-3'-acetylamide-1'-anilide in sufficient amount to effectively absorb ultra-violet rays.

15 10. A sheet material permeable to ultra violet rays containing a compound, substantive to said sheet material, selected from the class consisting of diaminodibenzoyl compounds of p-phenylenediamine disulfonic acid, p-phenylenediamine sulfonic acid and 3,6-diaminocarbazole disulfonic acid, the sodium salt of 4,4'-tetramethyldiamino-dibenzoyl-4,4'-diamino-diphenyl-2,2' disulfonic acid and substitution products thereof, the sodium salt of di-m-amino-benzoyl-diaminostilbene disulfonic acid, the arylides of 2,3-hydroxynaphthoic acid, the arylides of 2,3-hydroxynaphthoic-aminosulfonic acid, salicyl-p'-aminosalicyloyl-m''-aminophenol, 3-hydroxy-diphenylamine, m-aminoanilide of 3-hydroxy-4'-chlorodiphenylamine carboxylic acid, (1,2,5-trichlorobenzene-4-sulfo)-(4',6'-dichloro-1'-phenol-2'-sulfo)-1',3''-phenylenediamine, and 4-chloro-1-phenol-2,6-disulfo-bis-3'-acetylamide-1'-anilide in sufficient amount to effectively absorb ultra-violet rays.

20 11. A process as defined in claim 7 wherein the sheet material is a cellulosic material.

25 12. A process as defined in claim 8 wherein the sheet material is a cellulosic material.

30 13. A product as defined in claim 9 wherein the sheet material is a cellulosic material.

35 14. A product as defined in claim 10 wherein the sheet material is a cellulosic material.

JOHN EGGERT.  
BRUNO WENDT.